

## UNITED STATES PATENT OFFICE

JOHN C. BLACK, OF LOS ANGELES, WIRT D. RIAL, OF LOS ANGELES COUNTY, AND JOHN R. McCONNELL, OF WHITTIER, CALIFORNIA, ASSIGNEES, BY MESNE ASSIGNMENTS, TO RICHFIELD OIL COMPANY OF CALIFORNIA, OF LOS ANGELES, CALIFORNIA, A CORPORATION OF DELAWARE

## PROCESS OF IMPARTING A GREEN FLUORESCENCE TO LUBRICATING OIL

No Drawing.

Application filed May 18, 1927. Serial No. 182,476.

This invention relates to a method of extracting green fluorescent bodies from coal tar, coal tar distillates, or coal tar pitch with a solvent, and then utilizing the solvent containing the extracted green fluorescent bodies for improving the quality or imparting a desired green fluorescence to a lubricating oil stock. This application is a continuation in part of the application of John C. Black, 5 Wirt D. Rial and John R. McConnell, Serial No. 141,424, filed October 13, 1926, process of imparting fluorescence to oil.

As stated in that pending application, the trade associates a green fluorescent lubricating oil stock with quality, therefore it is desired for commercial reasons to impart a green fluorescence to certain grades of lubricating oil stock.

It is generally known to those skilled in 20 the art, that certain lubricating oil stocks without this green fluorescence may contain an undesirable fluorescence, and that this undesirable fluorescence usually is characteristic of a stock which has been derived by distillation of any crude petroleum oil.

In the manufacture of lubricating oil from crude petroleum oil free from asphalt, or substantially free from asphalt, a green fluorescence will result in the residuum remaining 25 after the removal of the lower boiling oils, even though the residuum has been subjected to a light cracking operation to crystallize the amorphous wax contained therein, and a lubricating oil stock can be produced from the same with a green fluorescence. Also a lubricating oil with a green fluorescence can be made by acid treating an asphalt base oil residuum if sufficient acid is employed to remove substantially all the asphaltic content. 30 However, such methods are impracticable since very large amounts of acid must be used, thus entailing low yields of the finished lubricating oil.

It is an object of this invention to extract 45 green fluorescent bodies from a coal tar, coal tar pitch or distillates of the same with a solvent and then utilize the solvent containing the extracted green fluorescent bodies for improving the quality or imparting a desired green fluorescence to lubricating oil stocks,

so that the lubricating oil stock will not be characterized by an undesirable color when viewed by reflected light, but will be generally characterized by a green fluorescence, and will be further characterized by a red, 55 reddish brown, yellow, or shades of yellow when viewed by transmitted light.

We have found that certain bodies extracted from coal tar, coal tar pitch, or distillates of the same, will impart to a lubricating oil 60 stock a green fluorescence.

The process of this application consists in concentrating these green fluorescent bodies in a solvent or medium, and then commingling the concentrated extract with a lubricating oil stock in quantities sufficient to produce the desired green fluorescence. It is an important advantage of this process that by employing a concentrated fluorescent extract, substantially no impurities associated 65 with the fluorescence material are introduced into the oil.

As an example of suitable materials from which green fluorescent bodies may be extracted for imparting a desired green fluorescence to a lubricating oil stock, coal tar, 70 coal tar pitch, or high boiling distillates of the same may be used. A coal tar pitch which does not contain low boiling hydrocarbons is preferred, although coal tar or 75 coal tar pitch containing small percentages of low boiling hydrocarbons may be employed, and the low boiling hydrocarbons 80 eliminated by distillation, preferably after the extraction process and before the addition to the lubricating oil stock. However, 85 it is to be understood that this elimination of the low boiling hydrocarbons, if any is contained therein, may be carried out after the addition of the fluorescent extract to the 90 lubricating oil stock by a subsequent distillation or reduction operation.

The solvent or medium to be employed for extracting the green fluorescent bodies may be any pure hydrocarbon, such, for example, as gasoline, benzol, and the like, or preferably a high boiling petroleum oil such as a lubricating oil stock. When employing volatile solvents, the extract is made by commingling comminuted coal tar pitch with 95 100

the solvent, preferably near the boiling point of the solvent. The extract in the required proportions is added to the lubricating oil stock and the solvent removed by 5 volatilization.

We have found it more desirable, however, to employ high boiling hydrocarbon oils such for example, as a lubricating oil having a flash point the same or higher than the lubricating oil stock to which the fluorescent extract is to be added. The solvent or medium, preferably lubricating oil stock, is commingled with approximately 1 to approximately 25 per cent by weight of coal tar pitch or 10 other high flash coal tar residues which contain extractable green fluorescent bodies, at a temperature of approximately 230 to 300 degrees F., and preferably in the presence of a decolorizing clay which will absorb 15 all the undesired constituents of the petroleum oil pitch, and also act as a filter medium to prevent any finely comminuted particles from passing through with the solvent or medium. In case a decolorizing clay is not 20 employed in the manufacture of the extract, which is used for imparting a desired green fluorescence to the lubricating oil stock, it may be added directly to the lubricating oil stock to which the fluorescent bodies are to 25 be added, and thereafter clarified and decolorized to the desired degree by methods well known in the art.

In case a volatile solvent or medium is employed, approximately the same amount of 30 coal tar pitch, coal tar, or coal tar distillate, that is, from 1 to as high as 25 per cent by weight, or higher, is employed at a temperature preferably near the boiling point of the solvent or medium, although normal temperatures may be employed with such solvents as benzol or gasoline. After the petroleum pitch has been commingled at the required temperature with the solvent or medium, which may or may not have been filtered 35 in the presence of a decolorizing clay, this concentrated extract is then added in the required amount to the lubricating oil stock, to which the desired fluorescence is to be imparted, and the volatile solvent separated by 40 a distillation operation, or the lubricating oil stock commingled with the concentrated fluorescent extract may be first clarified and decolorized by means of a decolorizing agent, and the volatile solvent thereafter separated by distillation. In case a coal tar distillate is employed that fraction known as 45 "middle oil" is preferably used, and preferably having boiling points ranging from approximately 400 to 600 degrees F.

As a specific example of obtaining a green 50 fluorescent extract from coal tar pitch suitable for imparting a green fluorescence to lubricating oil, a coal tar pitch having a penetration of approximately 2 was dissolved in benzol, approximately at the rate 55

of 25 parts of oil pitch to 75 parts of benzol. This mixture was then treated with sulfuric acid in quantities sufficient to precipitate substantially all the asphaltic material contained therein. After the removal of the precipitated asphalt and products of the acid reaction, a green fluorescent extract was obtained in a benzol solution. After removal of the benzol by distillation there was produced a concentrated green fluorescent extract suitable for producing the desired green fluorescence when added to a lubricating oil stock. In like manner a lubricating oil stock may be used as the solvent instead of benzol. 70 75

In the preferred method of operating this invention, the lubricating oil stock is preferably acid treated before the addition of the concentrated green fluorescent extract, after which the sludge is removed, and the acid treated oil is then commingled with the required amount of concentrated green fluorescent extract, which is also preferably an acid treated lubricating oil stock containing a high percentage of green fluorescent bodies made in the manner heretofore described. 80 85 The commingled lubricating oil stock containing the green fluorescent extract is then clarified and decolorized by well-known methods. 90

By the term "solvent" or "medium", we 95 mean an oil which will dissolve or retain in a colloidal suspension the green fluorescent bodies from a coal tar pitch.

While the process herein described is well adapted for carrying out the objects of the present invention, it is to be understood that various modifications and changes may be made without departing from the spirit of the invention and the invention includes all such changes and modifications as appear in the scope of the appended claims. 100 105

We claim:

1. A process of simultaneous refining and imparting a desired green fluorescence to a lubricating oil which is lacking in the same, comprising commingling a lubricating oil with a hydrocarbon oil containing green fluorescent bodies extracted from a coal tar residuum. 110

2. A process of simultaneous refining and imparting a desired green fluorescence to lubricating oil which is lacking in the same, comprising commingling a lubricating oil with a hydrocarbon oil containing green fluorescent bodies extracted from a coal tar pitch, and then separating the hydrocarbon oil from the lubricating oil and green fluorescent bodies. 115 120

3. A process of simultaneous refining and imparting a desired green fluorescence to lubricating oil which is lacking in the same, comprising commingling a lubricating oil with a hydrocarbon oil containing green fluorescent bodies extracted from a coal tar pitch, and then separating the hydrocarbon 125 130

oil from the lubricating oil and green fluorescent bodies, by distillation.

4. A process of simultaneous refining and imparting a desired green fluorescence to lubricating oil, which is lacking in the same, comprising extracting green fluorescent bodies from a coal tar pitch with a hydrocarbon oil, commingling the same with a lubricating oil and a decolorizing clay at temperatures sufficient to clarify and decolorize the lubricating oil and hydrocarbon oil containing the green fluorescent bodies, and then separating the clarified and decolorized lubricating oil containing the hydrocarbon oil and green fluorescent bodies from the decolorizing clay and adsorbed constituents.

5. A process for the manufacture of lubricating oil with a desired green fluorescence, comprising dissolving a coal tar pitch containing green fluorescent bodies in a solvent having a boiling point range substantially less than the lubricating oil, treating the solution containing the dissolved coal tar pitch with sulfuric acid in quantities sufficient to combine with substantially all of the carbonaceous content; separating the solvent containing the green fluorescent bodies from the acid reaction products; separating by distillation the solvent from the green fluorescent bodies and finally commingling the concentrated green fluorescent extract with a lubricating oil.

6. A process for the manufacture of lubricating oil with a desired green fluorescence, comprising dissolving a coal tar pitch containing green fluorescent bodies in a solvent having a boiling point range substantially less than the lubricating oil, treating the solution containing the dissolved coal tar pitch with sulfuric acid in quantities sufficient to combine with the major portion of the carbonaceous content; separating the solvent containing the green fluorescent bodies from the acid reaction products, commingling the solvent containing the green fluorescent bodies with a lubricating oil stock, separating by distillation the solvent from the lubricating oil and green fluorescent bodies, and finally clarifying and decolorizing to the required degree.

7. A process for the manufacture of lubricating oil with a desired green fluorescence, comprising dissolving a coal tar pitch containing green fluorescent bodies in a solvent hydrocarbon oil having a boiling point range substantially the same as the lubricating oil, treating the solution containing the dissolved coal tar pitch with sulfuric acid in quantities sufficient to combine with substantially all the black carbonaceous material contained therein, separating the solvent containing the green fluorescent bodies from the acid reaction products, and finally commingling the solvent containing the green fluorescent bodies with a lubricating oil.

8. A process for the manufacture of lubricating oil with a desired green fluorescence, comprising dissolving a coal tar pitch containing green fluorescent bodies in a lubricating oil, treating the lubricating oil containing the dissolved coal tar pitch with sulfuric acid in quantities sufficient to combine substantially with all the black carbonaceous content, separating the lubricating oil containing the green fluorescent bodies from the acid reaction products, commingling the lubricating oil containing the green fluorescent bodies with other lubricating oil, which is lacking in green fluorescent bodies, and a decolorizing clay at temperatures substantially not less than 230° F. and finally separating by filtration the combined lubricating oils containing the green fluorescent bodies from the decolorizing clay and adsorbed constituents.

9. A process of simultaneous refining and imparting a desired green fluorescence to lubricating oil which is lacking in the same, which comprises dissolving a high flash coal tar distillate in a hydrocarbon oil, commingling the same with a lubricating oil and a decolorizing clay at temperatures sufficient to clarify and decolorize the lubricating oil and the hydrocarbon oil containing the dissolved high flash coal tar distillate and green fluorescent bodies, and then separating the clarified and decolorized lubricating oil containing the hydrocarbon oil, high flash coal tar distillate and green fluorescent bodies from the decolorizing clay and adsorbed constituents.

10. A process for the manufacture of lubricating oil with a desired green fluorescence, comprising dissolving a coal tar distillate containing green fluorescent bodies in a solvent having a boiling point range substantially less than the lubricating oil, treating the solution containing the dissolved coal tar distillate with sulfuric acid in quantities sufficient to combine with a major portion of the colored carbonaceous material; separating the solvent containing the green fluorescent bodies from the acid reaction products; commingling the solvent containing the green fluorescent bodies with the lubricating oil stock; separating by distillation the solvent from the lubricating oil and green fluorescent bodies and finally clarifying and decolorizing to the required degree.

11. A process for the manufacture of lubricating oil with a desired green fluorescence, comprising dissolving a coal tar distillate containing green fluorescent bodies in a solvent hydrocarbon oil having a boiling point range substantially the same as the lubricating oil, treating the solution containing the dissolved coal tar distillate with sulfuric acid in quantities sufficient to combine with substantially all the colored carbonaceous material; separating the solvent contain-

- ing the green fluorescent bodies from the acid reaction products, and finally commingling the solvent containing the green fluorescent bodies with the lubricating oil.
- 5 12. A process for the manufacture of lubricating oil with a desired green fluorescence, comprising dissolving a coal tar distillate containing green fluorescent bodies in a lubricating oil, treating the lubricating oil
- 10 containing the dissolved coal tar distillate with sulfuric acid in quantities sufficient to combine substantially with all the colored carbonaceous material; separating the lubricating oil containing the green fluorescent
- 15 bodies from the acid reaction products, commingling the lubricating oil containing the green fluorescent bodies with other lubricating oil, which is lacking in green fluorescent bodies, and a decolorizing clay at tempera-
- 20 tures substantially not less than 230° F., and finally separating by filtration the combined lubricating oil containing the green fluorescent bodies from the decolorizing clay and adsorbed constituents.
- 25 In testimony whereof we affix our signatures.

JOHN C. BLACK.  
WIRT D. RIAL.  
JOHN R. McCONNELL.

30

35

40

45

50

55

60

65